

# UNITED STATES PATENT OFFICE.

ALEXANDER S. RAMAGE, OF DETROIT, MICHIGAN, ASSIGNOR TO CHEMICAL DEVELOPMENT CO., OF BUFFALO, NEW YORK, A CORPORATION OF COLORADO.

## METHOD OF SEPARATING MINERALS.

967,671.

Specification of Letters Patent. Patented Aug. 16, 1910.

No Drawing.

Application filed December 12, 1908. Serial No. 467,153.

To all whom it may concern:

Be it known that I, ALEXANDER S. RAMAGE, a citizen of the United States, residing at Detroit, in the county of Wayne and State of Michigan, have invented certain new and useful Improvements in Methods of Separating Minerals, of which the following is a specification.

The object of this invention is the provision of a method whereby a mineral may be separated from the gangue material, or one or more component minerals of a complex mixture may be successively separated, by hydrometallurgical or "flotation" processes.

It is well known that certain minerals, as for instance the sulfids of zinc, lead and iron may be separated from the gangue material by flotation in acid solutions, the liquids more commonly employed being heated solutions of sulfuric acid or acid sulfates. I have discovered that under proper conditions as hereinafter set forth it is possible to effect a successive separation of several mineral components of a complex mixture or ore by appropriately varying the conditions existing in a single solution. In order to accomplish this result I make use of a solution containing a constituent capable of reacting selectively, at proper temperatures, upon one or more of the component minerals.

In order that the invention may be fully understood I will describe the same by reference to a specific example, it being understood that the invention is not restricted to the conditions specified in this example. In the case of an ore containing sulfids of zinc, lead and iron I may employ a 10% solution of sodium nitrate or Chile saltpeter, together with sulfuric acid, yielding free nitric acid and acid sodium sulfate. The pulverized and properly graded ore is subjected to this solution at a temperature of approximately 140° F., whereupon the zinc sulfid rises to the surface in the form of a spongy mass which may readily be skinned off. The temperature is then raised to approximately 180° F., whereupon the iron sulfid rises to the surface and may be similarly removed, leaving a mixture of galena with the gangue material. This galena may be readily separated by known concentration methods. Under proper conditions there is no substantial solution of the minerals and with care a nearly perfect separa-

tion, amounting in some cases to 98%, may be secured. The liquor is used repeatedly, replacing the necessary losses of nitrate and sulfuric acid. The peculiarity of this separation is that the zinc sulfid rises in a sponge-like mass which can be readily washed from any mechanically entangled compact pyrites. The solutions may be more or less concentrated than above described, the temperature most favorable for the separation varying with the concentration of the solution.

For separating the above-described minerals, a solution of sodium chlorid and sulfuric acid may also be used, but the separation is somewhat less rapid and complete. The nitric acid solution is also highly effective in the separation of chalcocite and chalcopyrite.

The presence of limestone, dolomite, or similar materials will naturally result in the consumption or loss of considerable quantities of acid, and in case such compounds are present the ores may be subjected to a preliminary acid treatment, preferably with hydrochloric acid. In case fumes of sulfur dioxide are available from roasting furnaces, the hydrochloric acid is conveniently prepared by passing these fumes over sodium chlorid in heated cylinders in the well-known manner. Even when the amount of carbonates present is but small, it is desirable to decompose them by an acid treatment in order that no carbon dioxid may be evolved during the flotation, inasmuch as this gas appears to render the separation less exact by acting indiscriminately on the several mineral components.

While it is impractical to state definite temperatures or concentrations which are effective in bringing about the desired separation in all cases, the separation may be very readily and simply accomplished by slowly increasing the temperature of the solution to the point at which one mineral component floats, and maintaining the solution at or near this temperature, or below the temperature at which the second component rises, until the first component is removed. A further rise of temperature will then bring about the separation of the second component. In general, the solution should not be heated to a temperature substantially above that at which a given separation occurs until the separated component has been removed.

In case of free metals I may use the above named solutions, or a solution of sodium chlorid or sodium sulfate containing free caustic soda. The process is likewise applicable to the separation of a single mineral from a gangue material. For example I have found that zinc sulfid disseminated through a gangue of dolomite may be successfully treated as follows: The ore is first mechanically concentrated, say to a 30% concentrate, and is then immersed in a high-gravity solution containing for example 10% of sodium nitrate to which sulfuric acid has been added, preferably in proportion to form acid sodium sulfate. Effervescence occurs at first but ceases in a short time as the gangue material becomes coated with sulfate. At a temperature approximating 140° F., the zinc sulfid is found to rise with substantial completeness, an examination of the gangue showing only 0.22% of zinc remaining therein. The acid liquid in this case reacts directly with the mineral particles, enveloping them in a gaseous sheath or envelop by which they are elevated. For the best results the ore should be ground to number ten mesh or finer, as if the particles are larger than this

there is a tendency for the gas to escape in the form of bubbles without exerting its full efficiency in raising the mineral. 30

I claim:—

1. The method of treating ores containing a plurality of mineral components, which consists in immersing the ore in a suitable solution, separately floating said mineral components by progressively raising the temperature of the solution, and removing at each rise of temperature the product separated during such rise. 35

2. The method of treating ores containing a plurality of mineral components, which consists in immersing the ore in a suitable solution containing free nitric acid, separately floating said mineral components by progressively raising the temperature of the solution, and removing at each rise of temperature the product separated during such rise. 45

In testimony whereof, I affix my signature 50 in presence of two witnesses.

ALEXANDER S. RAMAGE.

Witnesses:

CHARLES H. POTTER,  
N. P. LEONARD.